

June 6, 1933.

N. S. CLAY

1,912,931

MOLDED ARTICLE

Filed May 17, 1928

4 Sheets-Sheet 1

Fig. 1.



Fig. 2.



INVENTOR

Noble S. Clay.

BY  
Shelley S. Carr

ATTORNEY

June 6, 1933.

N. S. CLAY

1,912,931

MOLDED ARTICLE

Filed May 17, 1928

4 Sheets-Sheet 2

Fig. 3.



Fig. 4



Fig. 5.

INVENTOR  
Noble S. Clay.

BY  
Wesley E. Barr  
ATTORNEY

June 6, 1933.

N. S. CLAY

1,912,931

MOLDED ARTICLE

Filed May 17, 1928

4 Sheets-Sheet 3



INVENTOR  
Noble S. Clay.

BY  
Burley & Barr  
ATTORNEY

June 6, 1933.

N. S. CLAY

1,912,931

MOLDED ARTICLE

Filed May 17, 1928

4 Sheets-Sheet 4



Fig. 9.



Fig. 12.



Fig. 10.



Fig. 13.



Fig. 11.

INVENTOR  
Noble S. Clay

By  
Bentley & Barr  
ATTORNEY

## UNITED STATES PATENT OFFICE

NOBLE S. CLAY, OF WILKINSBURG, PENNSYLVANIA, ASSIGNOR TO WESTINGHOUSE ELECTRIC & MANUFACTURING COMPANY, A CORPORATION OF PENNSYLVANIA.

## MOLDED ARTICLE

Application filed May 17, 1928. Serial No. 278,513.

My invention relates to composite products and it has particular reference to trays of composite material that are particularly adapted to cafeteria service. Most trays of the prior art have been made of certain metallic materials, such as aluminum and the like. Trays made of this material have the disadvantage that they are noisy, oxidize readily and that dirt clings to their surfaces. 10 It is, therefore, an object of my invention to provide a tray in which the above disadvantages are entirely obviated.

Another object of my invention is to provide a tray which is pleasing to the eye and 15 permits of ornamentation.

Still another object of my invention is to provide a tray which is sturdy in construction and low in cost of manufacture.

After considerable experimentation, I have 20 succeeded in producing a tray made of laminated material consolidated with a heat-hardened binder and find that the tray so produced has especially desirable characteristics.

The invention may be better understood by 25 reference to the accompanying drawings, in which,

Figure 1 is a view, in perspective, of a finished tray made according to my method of manufacture,

30 Fig. 2 is an exploded view of the sheets of treated material as they are assembled preparatory to molding according to one of my methods of manufacture,

Fig. 3 is a view, partly in elevation and 35 partly in section, of the dies of a press, with the necessary material assembled therein, preparatory to the molding of a tray,

Fig. 4 is a view, partially in elevation and 40 partially in section, of the dies of a press and the tray during the process of molding,

Fig. 5 is a view, in section, of a part of the tray, showing the upturned flange portion, and manufactured according to one of my methods of manufacture,

45 Fig. 6, Fig. 7 and Fig. 8 show portions of the dies of a press, together with the necessary material, for making trays according to a modified method of manufacture,

Fig. 9 is a view, partly in top elevation and 50 partly in section, taken along the line

IX—IX of Fig. 10, and showing a tray made according to a modified method of manufacture,

Fig. 10 is a view, in section, of a portion of a tray made according to a modified method 55 of manufacture,

Figs. 11 and 12 are views, in elevation, illustrating examples of methods of cutting the corners of the sheets in order to avoid excess material at the corners of finished trays, 60 and;

Fig. 13 is a view, in perspective, showing a method of forming the sheets preparatory to molding, in order to avoid excess material at 65 the corners of the finished tray.

Referring more particularly to Figs. 1 and 2, I have found it desirable to make the tray 1 of a plurality of layers of suitable treated fibrous material, such as paper, cloth and the like. Treated fibrous material, in a 70 shredded or chopped condition, may also be used. The preferred treating material or impregnating binder is a phenolic condensation product, although other binders capable of being hardened under the action of heat may 75 be utilized.

Sheets of different dimensions may be utilized, as, for instance, a preferred structure would embody four sheets 2 of treated paper for the bottom cover, four body or filler sheets 80 3 of the same size as the bottom of the finished tray, four body or filler sheets 4 of a size intermediate that of sheets 2 and sheets 3 and four full-size upper-cover sheets 5. The cover sheets 2 and 5 are preferably treated with a 85 higher content of binder than are the sheets in the interior of the tray.

If desired, inserts, such as strips of material 6, or pieces of treated or untreated rope, wires or the like may be utilized to provide 90 a thicker edge portion or lip for the tray. These strips are arranged in the form of hollow rectangles, and the corners thereof may be reinforced by special reinforcing sheets, 95 such as the triangular corner pieces 7. Furthermore, various shaped pieces of material, such as triangular pieces, may be removed from the corners of certain of the sheets as shown in Fig. 11, or the corners may be slotted (Fig. 12) to provide strips of material which 100

may be overlapped as shown in Fig. 13, to permit better fitting of the sheets in the mold and reduce the amount of material at the corners of the finished tray.

- 5 If desired, small insignia sheets 8, (Figs. 1 and 2) on which various designs are printed, may be placed either just inside the bottom surface layers or under the top surface layers. As an alternative, full-size surface-sheets 10 upon which the insignia is printed may be utilized. After the hardening treatment, this insignia will be found to be plainly visible through the superposed material of the tray. In this manner, I may provide variously decorated or colored cover sheets in order to give the tray a decorative appearance, such as that obtained with highly polished wood finishes and the like. The trays are molded, under heat and pressure, 15 in the usual manner and any excess material at the corners trimmed away.
- The sheets are assembled in the order shown in Fig. 2 and stacked on the lower die 13 of the mold shown in Fig. 3, the sheets bending 20 downward at the center by reason of their own weight. The mold is closed, as in Fig. 4, and heat and pressure applied, in the usual manner, to harden the binder and consolidate the laminations. The closing of the mold 25 causes the edges of the various sheets to be crumpled together or conglomerated to fill the edge portions of the mold, thus providing the folded, thickened or conglomerated edge portion 22, shown in Fig. 5.
- 30 A modified method of manufacture is shown in Figs. 6, 7 and 8. In this process, the sheets of treated material 11 are all of the same size, the dimensions being such that the sheets are slightly larger than the total lower 35 surface area of the finished tray. Preferably, sixteen sheets are utilized but, of course, any other number of sheets may be employed, according to the character of the material and the desired thickness of the finished article.
- 40 Special dies, such as the dies 12 and 13 shown in Fig. 6, are employed. The upper die 12 is recessed at its outer portion 14, so that a hollow rectangular member 15 may be placed on the lower die between the flanges 16 45 and 17. The rectangular member 15 is provided, at its upper inner edge, with a ledge 18 large enough and deep enough to receive the sheets of treated material, and it is further provided with an inner surface portion 19 sloping downwardly and inwardly therefrom.

In making a tray according to the second method, the treated sheets are placed on the ledge 18 of the rectangular member 15 of the dies. The mold is then closed. This action pushes the sheets into the recess 20 of the lower mold, bending them upwardly at the edges (Fig. 7). Since the weight of the sheets causes them to bend downwardly at the middle, (Figs. 6 and 7) the slightly over-

size sheets are entirely contained in the opening between the dies. As the mold is closed, the convex portion 21 of the sheets is flattened out, and the excess sheet material forced into the side wall opening of the mold, where it is scraped down the wall 19 of the rectangular member 15 and crumpled and folded to provide the thick beaded edge portion 22 of the tray.

The corner wall openings (not shown) between the dies of the mold are of greater thickness so that the excess material at the corners of the sheets may be crumpled and folded, in the same manner as the bead, to provide a thicker wall section 23 (Fig. 9) of folded or conglomerated material at the corners of the tray to better withstand shock, and in order to permit the utilization of ordinary sheets without cutting out certain portions, as has been hitherto described. Molding under heat and pressure is then carried on, in the usual manner, to complete the process. The corner portion of a tray made according to this process is shown in Figs. 9 and 10.

I have found, in manufacturing the trays, that great care must be used in the treatment of the sheet material and that, if the treating operation and molding operation are not carefully practiced, blisters are likely to form after the molding operation. I have found that this difficulty may be obviated by close attention to the operation of treating the sheet material.

It has been found that blistering is ordinarily caused by the volatile matter included in the binder and that, if the sheets, prior to molding, are carefully dried at a temperature of from 90 to 120° for from 10 to 30 minutes, this difficulty is obviated. The cover sheets, the binder content of which is relatively high, must be closely watched, as regards the volatile matter inclusion. If the inclusion is kept under 4%, blistering is not likely to occur.

A tray made according to my method of manufacture will be found to be easy to clean, noiseless, pleasing to the eye and low in cost of manufacture.

Although I have described certain preferred processes and structures, it is apparent that further modifications may be made by those skilled in the art without departing from the spirit and scope of my invention as defined in the appended claims.

I claim as my invention:

1. The process of forming trays which comprises placing fibrous material impregnated with a binder capable of being hardened under the influence of heat and pressure, in the matrix of a mold in such a manner that a major proportion of the fibrous material rests upon the bottom of the mold and the remainder extends upwardly at an angle thereto, forming an edge portion having a

substantially flat upper surface, and simultaneously applying heat and pressure substantially perpendicular to the plane of the angular extending material and substantially vertical pressure to the material resting on the bottom of the mold and to the edge of the upwardly extending edge portion, sufficient pressure being applied to form a composite article having upwardly extending 5 side walls and an outwardly extending peripheral flange.

2. The process of forming trays which comprises assembling a plurality of lower surface sheets, a plurality of top surface sheets and a plurality of filler sheets having a smaller area than the surface sheets, forcing the assembly into a mold of such a shape and contour that the margin of the surface sheets will be folded upwardly at an angle 15 to the filler sheets and then consolidating the mass under the influence of heat and pressure 20 to form a composite article.

3. The process of forming trays which comprises assembling a plurality of surface sheets and a plurality of filler sheets having less area than the surface sheets, bending the margin of the surface sheets upwardly at an angle to the filler sheets and simultaneously 25 exerting pressure on the filler sheets and main 30 portion of the surface sheets and upon the upwardly extending margin of the surface sheets to consolidate the material into a composite article.

4. The process of forming molded articles 35 which comprises assembling a plurality of filler sheets upon one or more surface sheets, folding the margin of the surface sheets upwardly at an angle to the filler sheet and applying pressure against the assembled 40 structure to consolidate it into a composite article.

5. The process of forming trays which comprises placing a plurality of filler sheets upon surface sheets having a greater surface 45 area than the filler sheets, folding the margins of the surface sheets upwardly to form a bottom, an angular disposed portion and a substantially flat upper edge and then applying sufficient pressure upon the various parts 50 to bend the edge portion outwardly at a direction substantially parallel to the bottom portion and to consolidate the sheets into a composite article.

6. The process of forming trays which 55 comprises assembling a plurality of fibrous surface sheets, impregnated with a binder capable of being hardened under the influence of heat and pressure, and a plurality of fibrous filler sheets having less area than the 60 surface sheets impregnated with a similar binding agent and one or more inserts, folding the margin of the surface sheets at an angle to the filler sheets, and consolidating the assembled and formed sheets under the 65 influence of heat and pressure.

7. The process of forming trays which comprises assembling a plurality of upper surface sheets, a plurality of lower surface sheets, and interposing a plurality of filler sheets having less area than the surface sheets 70 between the lower and upper surface sheets, all of said sheets being impregnated with a binder capable of being hardened under heat and pressure, folding the margin of the surface sheets upwardly, thereby forming angularly disposed walls and a substantially flat edge, and then simultaneously applying heat and sufficient pressure to the bottom, the angularly disposed walls and the upper edge 75 to force the material at the edge outwardly to form a peripheral flange and to consolidate the material into a composite article.

8. The process of forming trays which comprises impregnating a plurality of upper surface sheets and a plurality of lower surface sheets with a comparatively large amount of a binding agent capable of being hardened under the influence of heat and pressure and a plurality of filler sheets impregnated with a less quantity of the binding agent than the surface sheets, bending the margins of the surface sheets at an angle 80 to the filler sheets and then applying pressure against the bottom and angularly extending side walls to form a rigid, composite article.

9. The process of forming trays which comprises impregnating a plurality of sheets of fibrous material with a binder capable of being hardened under the influence of heat and pressure, rounding the edges of the sheets, cutting out notches, thereby forming strips at the corners, folding the margin of the sheets upward at an angle to the main body portion, thereby causing the strips to abut against each other, assembling a plurality of such sheets and then simultaneously applying pressure against the bottom portion and the angularly disposed margin to form a composite article.

10. The process of forming trays which comprises impregnating a plurality of sheets of fibrous material with a binder capable of being hardened under the influence of heat and pressure, rounding the corners of the sheets, cutting notches out of the corners to form strips, assembling a plurality of such sheets and bending the margin upwardly, thereby causing the strips to abut against each other and form a substantially level edge, and simultaneously applying heat and sufficient pressure to the main portion of the sheets, the angularly extending portion and the edge portion to form a composite article having a bottom, upwardly inclined side walls and an outwardly projecting peripheral flange.

11. The process of forming trays which comprises impregnating a plurality of sheets of fibrous material with a binder capable of

- being hardened under the influence of heat and pressure, rounding the corner portions, cutting slits in the corners to form strips, bending the margin of the sheets at an angle
- 5 to the main body portion and overlapping the strips formed at the corner, assembling a plurality of such sheets and applying heat and pressure to the bottom and the angularly bent portion to form a composite article.
- 10 12. The process of forming trays which comprises impregnating a plurality of sheets of fibrous material with a binder capable of being hardened under the influence of heat and pressure, rounding the corners of the
- 15 sheets, cutting slots therein to form a plurality of strips, assembling a plurality of such sheets, bending the margin upwardly at an angle to the body and overlapping the strips at the corners to form a substantially
- 20 level edge, then applying sufficient pressure to the bottom portion, the angularly disposed portion and the upper edge to force the material in the edge outwardly and to form a composite article having a bottom, an angularly disposed wall and an outwardly extending peripheral flange.
- 25 In testimony whereof, I have hereunto subscribed my name this 14th day of May, 1928.

30

NOBLE S. CLAY.

35

40

45

50

55

60

65